

## UNITED STATES PATENT OFFICE

2,067,507

PROCESS OF TREATING LEAD AND  
LEAD ALLOYSGeorge O. Smith, East Orange, N. J., assignor to  
Bell Telephone Laboratories, Incorporated, New  
York, N. Y., a corporation of New YorkNo Drawing. Application August 28, 1930,  
Serial No. 478,551

25 Claims. (Cl. 75—166)

This invention relates to a method of improving the mechanical properties of lead and lead alloys and more particularly to a method of alloying certain high melting-point metals 5 with lead or lead alloys at comparatively low temperatures.

A certain kind of commercial pig lead, such as Southeastern Missouri District lead, contains metallic impurities consisting of very small quantities of high melting-point metals, such as copper, silver, nickel and cobalt, and has been found to have physical properties which make this kind of lead especially desirable for certain purposes, as for example, for cable sheath alloys.

Another kind of commercial pig lead, such as Bunker Hill lead, has a high degree of purity and is particularly characterized by the almost total absence of the metals referred to above. This high purity lead has been found not to 20 possess the desirable physical properties to as high a degree as the first mentioned lead. It has furthermore been observed that when lead is alloyed with 1% of antimony, as for use in cable sheaths, the presence of the small quantity of high melting point metals has an additional advantageous effect upon the physical properties of the alloy.

The difference in physical properties may consequently be ascribed to the presence of the 30 metallic impurities referred to, which appear to impart to the lead as well as to the lead alloy greater tensile strength, higher percentage elongation, and better fatigue resisting properties.

In accordance with the invention a method is provided by which certain high melting-point metals, such as copper, silver, nickel and cobalt, may be added to lead or to certain lead alloys, such as antimony lead, at comparatively low 40 temperatures and in exact, small quantities to produce lead alloys with improved physical properties.

During an extensive investigation of lead and lead antimony alloys it was found that comparatively small quantities of oxides and certain salts, such as chlorides, of these high melting point metals are practically completely reduced in the presence of the lead or antimony under the application of heat, that is, the free metal present replaces and liberates the one contained in the salt or the oxide, at least in those instances where the heat of formation of the new salt or oxide is higher than that of the original 50 salt or oxide. Certain other salts of these metals,

such as bromides, fluorides, and iodides react similarly to the chlorides.

Thus, when small quantities of chlorides of high melting-point metals, such as copper, silver, nickel, cobalt and others, are added to a large 5 bath of molten lead, the lead replaces all of the high melting-point metal of the salt to form lead chloride and the liberated high melting-point metal then alloys with the lead. The required temperature for the reaction need only 10 be slightly above the melting point of lead chloride. Similar reactions take place when the chlorides are added either to a bath of molten antimony or to a bath of molten lead antimony alloy.

15 Certain oxides, which do not readily react with lead in a process such as that described, have been found to react with antimony in such a process. When copper oxide is in contact with molten lead at a temperature of approximately 20 500° C. metallic copper and lead oxide are formed and, when there is an excess of lead, an alloy of lead and copper results. Oxides of copper, cobalt, nickel and iron react similarly with molten antimony resulting in alloys which may be 25 used as addition products in the manufacture of lead antimony alloys containing these metals; or the oxides can be brought into contact with a lead antimony alloy whereupon, at a temperature of approximately 500° C., the antimony in 30 the alloy will reduce the oxides and the copper, cobalt, nickel and iron will enter the melt. The by-products of the reaction is antimony oxide.

An important feature of the method resides in the fact that practically the total amount of 35 metal added in the form of salt or oxide enters into the lead.

Another important feature resides in the fact that the process may be carried out at temperatures considerably below the melting points of 40 the metal to be added, the highest necessary temperature used in the process being not much above the melting point of lead. This fact is of advantage in a commercial process in that the process is simplified thereby and is made more 45 economical.

A further advantage observed in connection with the use of chlorides is due to the fact that lead chloride formed during the reaction is not 50 miscible with lead and therefore readily separates from the lead product without contaminating it. The lead chloride formed floats on the molten metal and serves as a flux. Certain other compounds of lead, such as lead phosphide and lead 55

sulphide do not possess the property of not contaminating the final product.

It is well known in the art to reduce metallic salts or oxides in the presence of other metals, 5 but the prior methods have either been in the nature of laboratory experiments, or the alloying constituents or the temperatures have been different from those used in the present process as defined by the appended claims.

10 In practicing the process in accordance with the invention, silver, copper, nickel and cobalt have been alloyed with lead by adding the chloride of these metals. Antimony has also been alloyed with silver, copper, nickel and cobalt 15 by the addition of the chlorides of these metals. Copper has been added to lead as well as to antimony by adding copper oxide to the metallic lead and antimony. The percentage of high melting point metal that may be added by this process 20 is different for the different metals and varies from less than .5% to a few percent of the lead or antimony.

In preparing these alloys one procedure was to melt pure lead and heat to 525° C. in a crucible, 25 remove the crucible from the furnace and skim the dross off the surface of the melt; the chlorides or oxides of the metals to be incorporated were then added; the molten metal was stirred and when its temperature was about 410° 30 C. the dross was removed again and the alloy was cast into molds.

Another procedure, which has been used successfully, involved the addition of 1% or slightly more of antimony to the molten lead; the process 35 was then continued as just described. In this procedure antimony chloride will be formed during the reaction instead of lead chloride, for which reason a loss of antimony must be anticipated.

40 Still another procedure, which has been used successfully involves the addition of one percent or more of antimony, either as metallic antimony or as an addition alloy of lead and antimony, to the molten lead immediately after the 45 small quantities of the other metals have been incorporated.

In some cases antimony was used instead of lead for alloying with the high melting-point metal, the procedure being substantially the same 50 as when lead was used and the resulting alloy was in turn added to lead.

It should be understood that other metals than those described may be added to lead or antimony by this process; for example, arsenic, 55 lead, bismuth, and iron may be added to antimony by means of their chlorides; arsenic may be added to lead by means of its chloride; and arsenic, bismuth, cobalt, iron, lead and nickel may be added to antimony by means of their 60 oxides.

It should also be understood that the process 65 may be varied from the described procedures. Thus the temperature may be increased considerably above 500° C., but for practical purposes it would not be advantageous to increase the temperature much beyond 600° C. It is also possible to add the ingredients to the lead or the antimony at ordinary room temperature 70 and then heat to about 500° C. It is also within the scope of the invention to add the chlorides of the desired metals to the lead in the mold, by, for example first placing the chlorides in the mold and then pouring the lead or lead alloy 75 into the mold, permitting the reaction to take

place in the mold by maintaining a sufficient casting temperature.

What is claimed is:

1. A method of alloying with a body of lead free of alkaline metals, another metal having 5 a higher melting point than that of lead and the chloride of which has a heat of formation less than that of lead chloride in an amount less than 5% by weight of the lead which comprises reducing a quantity of chloride of said metal in 10 a bath of said lead, free of alkaline metals, at a temperature between the melting point of said lead and 600° C., said quantity of chloride of said metal containing the approximate desired amount of said metal to be added. 15

2. A method of alloying a definite small quantity of copper with lead, which comprises adding together in a container lead, antimony and chloride of copper, both said lead and said antimony being free of alkaline metals, and maintaining the temperature of the contents of said 20 container at about 400° to 500° C. for at least a few minutes.

3. A method of alloying cobalt with lead in a desired amount of not more than .4% of the 25 lead which comprises maintaining a bath of molten lead, which is free of alkaline metals at a temperature not more than about 100° C. above the melting-point of lead chloride, and adding the amount of cobalt in the form of 30 cobalt chloride to the bath.

4. A method of alloying copper with lead in a desired amount of not more than 1% of the lead which comprises maintaining a bath of molten lead, free of alkaline metals, at a tem- 35 perature not more than about 100° C. above the melting point of lead chloride and adding the amount of copper in the form of copper chloride to the bath.

5. A method of alloying silver with lead in a 40 desired amount of not more than 1% of the lead, which comprises adding together lead, which is free of alkaline metals, and the amount of silver in the form of silver chloride and maintaining the lead at a temperature not more 45 than about 100° C. above the melting point of lead chloride for a few minutes after said adding.

6. A method of alloying silver and copper with lead in desired amounts each of not more than 1% of the lead which comprises adding together 50 lead, free of alkaline metals, and the amounts of silver and copper in the form of chlorides and maintaining the lead at a temperature not more than about 100° C. above the melting point of lead chloride for a few minutes after said adding. 55

7. A method of alloying with lead in a desired amount of not more than 1% of the lead which comprises maintaining a bath of molten lead, free of alkaline metals, at a temperature not more than about 100° C. above the melting point 60 of lead halide and adding the amount of copper in the form of a halide to the bath.

8. A method of improving the physical properties of lead by the addition thereto of a small quantity of a metal having a higher melting point 65 than that of lead, said method comprising adding to the lead, which is free of alkaline metals, a quantity of a compound comprising said metal and a non-metallic constituent selected from the group which consists of oxygen, fluorine, chlorine, 70 bromine and iodine, said compound having a lower heat of formation than the compound comprising lead and said non-metallic constituent, said last mentioned compound being not readily miscible with said lead and said lead being main- 75

tained at a temperature between the melting point of said lead and the boiling point of the compound comprising lead and said non-metallic constituent.

5 9. A method of improving the physical properties of alloys comprising chiefly lead by the addition thereto of small quantities of metal having a higher melting point than that of the alloy, said method comprising adding to the 10 alloy, which is free of alkaline metals, a desired quantity of the halide of said metal at a temperature between the melting point of said alloy and the boiling point of the corresponding halide of lead, said halide of said metal having a lower 15 heat of formation than said corresponding halide of lead and said halide of lead being not readily miscible with said alloy.

10. A method of improving the physical properties of lead alloy by the addition thereto of 20 small quantities of a metal having a higher melting point than that of the alloy, said method comprising adding to the alloy, which is free of alkaline metals, a desired quantity of the halide of said metal, said halide having a lower heat of 25 formation than the corresponding halide of lead, said halide of lead not being readily miscible with said alloy, and heating said mixture to a temperature approximately between the melting point of said lead halide and 100° C. higher.

30 11. The method of forming an alloy comprising copper and lead which comprises subjecting a molten bath maintained at a temperature below the boiling point of lead chloride and containing metallic lead, which is free of alkaline 35 metals, to the action of a chloride of copper thereby to effect the precipitation and dispersion of metallic copper in the molten bath.

12. A method of incorporating a metal having a higher melting point than that of lead in an 40 alloy comprising metallic lead, said method comprising subjecting a molten bath of said alloy to the action of a compound comprising said metal and a non-metallic constituent selected from the group which consists of oxygen, fluorine, 45 chlorine, bromine and iodine, said compound having a lower heat of formation than the compound comprising lead and said non-metallic constituent, said compound comprising said metal reacting with said metallic lead to disperse said 50 metal in said alloy and to form a compound comprising lead and said non-metallic constituent which is substantially non-miscible in said alloy in the absence of sufficient alkaline metals in said bath to introduce the desired amount of said high 55 melting point metal by the interaction of said alkaline metals with said compound comprising said high melting point metal, at a temperature below the boiling point of said compound comprising lead.

60 13. The method of forming an alloy comprising copper and lead which comprises subjecting a molten bath comprising metallic lead to the action of a compound comprising copper and a non-metallic constituent, said compound 65 having a lower heat of formation than the compound comprising lead and said non-metallic constituent, said compound comprising copper reacting with said metallic lead to form metallic copper and a compound comprising lead and 70 said non-metallic constituent which does not contaminate the resulting alloy in the absence of sufficient alkaline metals in said bath to introduce the desired amount of copper by the interaction of said alkaline metals with said 75 copper compound, said bath being maintained

at a temperature below the boiling point of said compound comprising lead and said non-metallic constituent.

14. The method of forming an alloy comprising copper and lead which comprises subjecting a molten bath of metallic lead, which is free of alkaline metals, to the action of an amount of copper chloride equivalent to about 1.2 pounds of copper per ton of lead in the bath said bath being maintained at a temperature below the 10 boiling point of lead chloride.

15. A method of alloying copper with lead comprising subjecting a chloride of copper to a molten bath of an alloy comprising lead and a metal other than a member of the alkaline group 15 which reacts with the chloride of copper to form metallic copper and the chloride of said metal, said bath being maintained at a temperature below the boiling point of lead chloride.

16. A method of forming a lead alloy comprising subjecting an alloy consisting of lead and elements having a higher melting point than that of lead to the action of a compound comprising a metal having a higher melting point than that of lead and a non-metallic constituent 25 selected from the group which consists of fluorine, chlorine, bromine and iodine and oxygen at a temperature between the melting point of said alloy and the boiling point of the compound comprising lead and said non-metallic constituent, said compound of said metal having a lower 30 heat of formation than the corresponding compound of lead.

17. A method of incorporating metals having a higher melting point than that of lead in lead, 35 said method comprising subjecting an alloy consisting of lead and elements having a higher melting point than that of lead to the action of the halide of a metal having a higher melting point than that of lead at a temperature between 40 the melting point of said alloy and the boiling point of lead halide, the halide of said metal having a lower heat of formation than the corresponding halide of lead.

18. A method of incorporating copper in lead 45 comprising subjecting a molten bath of an alloy consisting of lead and elements having a higher melting point than that of lead maintained at a temperature below the boiling point of lead halide to the action of a halide of copper whereby copper is dispersed throughout said alloy.

19. A method of incorporating a metal having a higher melting point than that of lead in an alloy comprising metallic lead, said method comprising subjecting a molten bath of said alloy 55 to the action of a halide of said metal in the absence of sufficient alkaline metals in said bath to introduce the desired amount of said high melting point metal by the interaction of said alkaline metals with said halide, said halide having a lower heat of formation than the corresponding lead halide at a temperature below the boiling point of said metal halide whereby said metallic lead reacts with said halide of said high melting point metal to disperse said metal 60 in said alloy and to form lead halide.

20. A method of alloying cobalt with lead which comprises adding together in a container lead, antimony and cobalt chloride, both said lead and said antimony being free of alkaline 70 metals, and maintaining the temperature of the contents of said container at about 400° C. to 500° C.

21. A method of alloying silver with lead which comprises adding together in a container lead,

antimony and silver chloride, both said lead and said antimony being free of alkaline metals, and maintaining the temperature of the contents of said container at about 400° to 500° C.

5 22. The method of forming an alloy comprising cobalt and lead which comprises subjecting a molten bath maintained at a temperature below the boiling point of lead chloride and containing lead which is free of alkaline metals to the action 10 of a chloride of cobalt thereby to effect the precipitation and dispersion of metallic cobalt in the molten bath.

15 23. The method of forming an alloy comprising silver and lead which comprises subjecting a molten bath maintained at a temperature below the boiling point of lead chloride and containing metallic lead which is free of alkaline metal to the action of silver chloride thereby to effect the

precipitation and dispersion of metallic silver in the molten bath.

24. A method of incorporating cobalt in lead comprising subjecting a molten bath of an alloy consisting of lead and elements having a higher melting point than that of lead and maintained at a temperature below the boiling point of lead halide to the action of a halide of cobalt whereby cobalt is dispersed throughout said alloy. 10

25. A method incorporating silver in lead comprising subjecting a molten bath of an alloy consisting of lead and elements having a higher melting point than that of lead and maintained at a temperature below the boiling point of lead 15 halide to the action of a halide of silver whereby silver is dispersed throughout said alloy.

GEORGE O. SMITH.